

## 1

2,898,222

## MANUFACTURE OF REGENERATED CELLULOSE

William R. Saxton and Bharat B. Mithel, Hawkesbury, Ontario, Canada, assignors to Canadian International Paper Company, Montreal, Quebec, Canada, a corporation of Quebec

No Drawing. Application January 30, 1956  
Serial No. 562,352

## 10 Claims. (Cl. 106—165)

This invention relates to new and useful improvements in the manufacture of regenerated cellulose from viscose into such articles as continuous filament tire yarn, textile yarn staple fibre, cellophane or sausage casings and the like, and particularly seems to provide a novel process in which the physical characteristics of the articles produced thereby are markedly superior to those obtained through the practice of previous processes.

In the production of viscose threads, cellulose, usually in the form of highly-refined dissolving wood pulp, is converted into alkali cellulose by treatment with caustic soda solution. The alkali cellulose so formed, after ageing, is converted into sodium cellulose xanthate by reaction with carbon disulphide. The sodium cellulose xanthate is dissolved in weak caustic soda solution to form the viscose solution. The viscose is then filtered, aged, and extruded through fine holes of a spinnerette into a spinning bath which normally consists of sulphuric acid and salts such as sodium sulphate and zinc sulphate. In the production of viscose threads for tire yarn the filaments thus formed are stretched in a plasticizing bath and are then treated with purifying solution, which in some cases may simply be hot water, and then are treated with a finish or sizing solution, and then are dried and wound into suitable packages.

We have now found that, under certain conditions of coagulation and regeneration of the viscose filaments in the spinning bath, a substantial difference in cross-sections and marked improvement in the physical properties of the yarn so formed can be achieved if there is present in the viscose in sufficient quantity one or more derivatives of ethylene oxide and aliphatic tertiary-alkyl primary amines. Such products have the generic formula:



where  $n$  is an integer between 4 and 50.

One such product which has been found satisfactory in the practice of this invention is "Priminox" as presently manufactured by Rohm & Haas Co.

Benefits will be conferred by 4 to 50 ethylene oxide units in the ethenoxy portion of these amide condensation products, but best results are obtained with 10 to 30 ethylene oxide units.

In accomplishing the objects of this invention we have found that it is necessary to incorporate in the viscose at least 1% by weight on the cellulose content of the viscose, and preferably 2% should be used. No further advantage can be obtained by using more than 4%.

The following examples will illustrate preferred embodiments of this invention, but the invention must not be construed as limited solely to these examples:

## EXAMPLE 1

Two percent, by weight based on the cellulose content of the viscose (oven dry basis), of derivatives of ethylene oxide and aliphatic tertiary-alkyl primary amines known commercially under the trademark "Priminox" were add-

## 2

ed to viscoses and spun into tire yarn under the conditions given below. In each case addition was made to the mixing solution before the xanthate was dissolved therein. In one case the additive was "Priminox 43" where  $n$ , the number of moles of ethylene oxide in the molecule, was equal to 1. In another case the additive was "Priminox 32" where  $n$ , the number of moles of ethylene oxide in the molecule, was equal to 25. A comparative untreated batch of viscose was also made and spun under identical conditions to the batches containing the additives.

Spinning conditions:  
 Viscose composition 7% cellulose, 6% NaOH  
 15 Ripening index, Hottenroth 30.  
 Ripening index, salt test 10.0.  
 Viscosity, ball fall 60-70 poises.  
 Spinning speed 50 metres/minute.  
 Denier 1650 (720 filaments).  
 20 Immersion of acid bath 28 inches.  
 Temperature of acid bath 60° C.  
 Acid bath composition  
 $\text{H}_2\text{SO}_4$  94.5 g./l.  
 $\text{ZnSO}_4$  122.7 g./l.  
 25 Density, 20° C. 1.274.  
 Percent stretch in second bath 80%.

The yarn so produced as twisted into a 2 ply cord of 11.35 Z/10.6 S turns per inch construction. Results 30 were as follows:

| 35 | Addition to Viscose | Denier | Grams/denier |             | Percent Elongation |             | Fatigue Life, Minutes |
|----|---------------------|--------|--------------|-------------|--------------------|-------------|-----------------------|
|    |                     |        | Oven Dry     | Conditioned | Oven Dry           | Conditioned |                       |
|    |                     |        |              |             |                    |             |                       |
| 0  |                     | 3,656  | 3.11         | 2.98        | 8.4                | 13.0        | 4.3                   |
| 2% | Priminox 43         | 3,692  | 2.89         | 2.89        | 7.9                | 12.9        | 0                     |
| 2% | Priminox 32         | 3,716  | 3.92         | 3.34        | 12.3               | 16.6        | 24.5                  |

It can be seen that the batch containing the additive "Priminox 43" where the number of moles of ethylene oxide in the additive molecule was only one, was actually inferior in cord properties to the control batch containing no additive whereas the batch containing the additive "Priminox 32" where the number of moles of ethylene oxide in the additive molecule was 25 gave cord 45 properties markedly superior to the control batch containing no additive. Furthermore, the cross-sections of the yarn produced from the batch containing "Priminox 32" were markedly different from those produced from the control batch.

50 The products may be added at almost any stage of the viscose process and even to the raw material cellulose itself if desired. However, for the accomplished purpose of the object of this invention we have found that addition to the mixing solution (the weak caustic soda solution used to dissolve the xanthate) before dissolution of the xanthate therein is the simplest and most efficient method.

55 Many variations of this process will suggest themselves to those skilled in the art, but such variations are considered as falling within the scope of this invention, provided the products employed are within the class described.

## We claim:

1. In the manufacture of regenerated cellulose by the 60 viscose process, the step of incorporating in the viscose from about 1% to about 4%, based on the weight of cellulose in the viscose, of derivatives of ethylene oxide

## 3

and aliphatic tertiary-alkyl primary amines having the generic formula



where  $n$  is an integer between 4 and 50.

2. The method of claim 1 in which the amount of derivatives of ethylene oxide and aliphatic tertiary-alkyl primary amines is about 1% based on the cellulose in the viscose.

3. The method of claim 1 in which the amount of derivatives of ethylene oxide and aliphatic tertiary-alkyl primary amines is about 2% based on the cellulose in the viscose.

4. The method of claim 1 in which  $n$  is 25.

5. In the manufacture of regenerated cellulose by the viscose process, the step of spinning viscose in the presence of from about 1% to about 4%, based on the weight of cellulose in viscose, of derivatives of ethylene oxide and aliphatic tertiary-alkyl primary amines having the generic formula



where  $n$  is an integer between 4 and 50.

6. The method of claim 5 in which the amount of derivatives of ethylene oxide and aliphatic tertiary-alkyl 25

10

20

primary amines is about 1% based on cellulose in viscose.

7. The method of claim 5 in which the amount of derivatives of ethylene oxide and aliphatic tertiary-alkyl primary amines is about 2% based on cellulose in viscose.

8. Viscose having incorporated therein from about 1% to about 4%, based on the weight of cellulose in the viscose, of derivatives of ethylene oxide and aliphatic tertiary-alkyl primary amines having the generic formula



where  $n$  is an integer between 4 and 50.

9. The method of claim 5 in which the amount of derivatives of ethylene oxide and aliphatic tertiary-alkyl primary amines is about 2% based on cellulose in viscose and in which  $n$  is 25.

10. The method of claim 1 in which  $n$  is an integer between 10 and 30.

## References Cited in the file of this patent

## UNITED STATES PATENTS

|           |                  |       |               |
|-----------|------------------|-------|---------------|
| 2,535,044 | Cox              | ----- | Dec. 26, 1950 |
| 2,593,466 | MacLaurin et al. | ----- | Apr. 22, 1952 |
| 2,710,861 | Charles et al.   | ----- | June 14, 1955 |